

May 26, 1931.

S. P. MILLER

1,807,223

METHOD OF FLAKING PITCH

Filed April 6, 1929



INVENTOR  
Street-Pamelle Miller  
BY  
Pauline Davis, Morris & Edwards  
ATTORNEYS

## UNITED STATES PATENT OFFICE

STUART PARMELEE MILLER, OF ENGLEWOOD, NEW JERSEY, ASSIGNOR TO THE BARRETT COMPANY, OF NEW YORK, N. Y., A CORPORATION OF NEW JERSEY

## METHOD OF FLAKING PITCH

Application filed April 6, 1929. Serial No. 352,990.

This invention relates to a new and improved method of solidifying pitch and similar substances such as certain resins, e. g. paracumarone resin, etc., which are brittle at lower temperatures and which become fluid at higher temperatures. More particularly this invention relates to a method producing flakes of pitch from fluid pitch, e. g. coal tar pitch, and is particularly adapted to flaking pitch of high melting point.

As is well known in the art, coal tar pitches, etc. are prepared for different uses in many degrees of hardness, running from those which are very soft and pliable at ordinary temperatures to those which are very hard and brittle at such temperatures. Although my invention may be applied to solidifying pitches or resins of various melting points, it is of particular value in handling coal tar pitches which are of sufficiently high melting point to be commonly sold or used in lump or crushed form.

Pitches are manufactured by subjecting tar to heat in a still and distilling off the required amount of oils to yield a residue of pitch which exists as a hot fluid mass which may be cooled to produce solid pitch of lower or higher melting point depending upon the degree of the distillation. The softer pitches, for example, those with a melting point up to about 160° F., are commonly sold in packages such as barrels due to the tendency of the softer pitches to agglomerate if made and handled in lumps or chips in bulk. Pitches of a melting point of 170-180° F. and above are, however, commonly produced and shipped in bulk as large lumps or even more or less finely crushed products. These harder pitches are ordinarily transferred to storage tanks while still hot and fluid and allowed to cool somewhat therein and then run into bays from which they must be excavated for shipment. The cost of excavating the pitch from bays and transferring it to suitable means for transporting it makes the use of bays expensive. The cooling of pitch by granulation in direct contact with water is sufficient but the removal of water from the pitch is difficult and expensive.

It is the purpose of my invention to over-

come the difficulties encountered by these various methods of handling pitch. Although, according to my invention, the pitch may be cooled in fact by direct contact with water, the cooling is preferably effected by indirect contact with water or other fluid cooling medium so that the pitch is produced in a dry form. The method is simple and entails little expense. The pitch is produced preferably in the form of thin flakes which can be handled easily. In this form pitch may be handled as a bulk product much as coal.

According to this invention, pitch, as it comes from the process of manufacture in a fluid heated state, may be solidified and formed directly into flakes, or pitch which has previously been produced in another form may be melted and converted into flake form.

The invention is particularly adapted to the handling of high melting point pitches such, for example, as those very high melting point pitches which may be produced in the distillation of tar by direct contact with hot coal distillation gases, although the invention is not limited to handling such pitches. It is particularly adapted to treating pitches of high melting point, such as pitches with a melting point of 400° F. or higher, or 350° F. or even lower melting point pitches, and is adapted to handling all pitches which are fluid at high temperatures and which, on cooling to near atmospheric temperature, are sufficiently brittle to be readily broken.

According to my invention the pitch in a molten condition is run on to the feed end of a conveyor, which is preferably a continuous metal belt. The belt is advantageously run over and driven by pulleys and the arrangement is preferably such that a considerable portion of the belt is positioned horizontally. The belt is kept in continuous motion, which may easily be done by driving one of the pulleys. The pitch in a fluid condition is run on to the upper belt surface at the feed end of the upper horizontal portions of the belt and the underside of this upper horizontal stretch of the belt is advantageously sprayed with water or other cooling medium so that the heat of the pitch is rapidly removed and the pitch

is solidified. The pitch is removed from the belt at or near the opposite end of the horizontal portion of the belt. Where the belt is run over two main pulleys, the pitch may advantageously be discharged from the belt as it passes over the pulley at the discharge end of the belt. Other means may be employed for discharging the pitch from the belt, such as scrapers or other side discharge means. 5 Where scrapers are employed, several hoppers or bins may be provided, positioned at different intervals along the length of the belt, so that as pitches of different melting points are produced, they may be discharged 10 to different hoppers or bins by changing the position of the discharge device. The highest melting point pitch which would be the first to solidify, would ordinarily be discharged into the hopper nearest the feed end 15 of the belt, and the lowest melting point pitch would ordinarily be discharged into the hopper nearest the discharge end of the belt. 20

The belt need not be horizontal. It may slope up or down from the point at which 25 the pitch is added. The degree to which the belt may slope will depend upon a number of factors, such as rate of addition of pitch, speed of belt, width of belt, temperature of pitch, temperature of cooling fluid, length of 30 belt, melting point of pitch, etc.

The pitch in a thinly fluid condition is fed on to the moving belt from a spout or other suitable discharge device and the rate of discharge of the pitch from the spout is co-ordinated 35 with the rate at which the belt moves so that the pitch forms on the belt as a sheet or ribbon which may vary in thickness. Ordinarily the operation is so controlled that a thin layer of pitch is formed which will cool rapidly. 40 As the pitch cools it becomes brittle and the pitch may shrink sufficiently to cause the ribbon of pitch on the belt to crack and form into several separate pieces. Means, such as a heavy roller, may be employed for comminuting 45 the pitch before it is discharged from the belt, although ordinarily no means for comminuting the pitch on the belt will be employed. Ordinarily the pitch will be broken sufficiently as it falls from the belt and 50 is collected in a suitable hopper or other collecting means.

This invention contemplates more particularly discharging the pitch from the belt as the belt passes over the pulley at the discharge 55 end of the belt. In passing over this pulley and discharging to the hopper the pitch which has been cooled sufficiently to make it brittle, is broken. The pitch is broken into flakes of irregular size and shape and may be 60 collected in bins or other suitable storage means.

The invention will be described further in connection with the accompanying drawings in which

65 Fig. 1 is a plan view of the apparatus;

Fig. 2 shows the apparatus in elevation; Fig. 3 is an end view; and Fig. 4 is a detail of the belt wiper.

In the drawings, 5 indicates the belt which may be a steel belt, preferably of rustproof 70 steel, or it may be Monel metal, bronze, etc. The high heat conductivity of the metal facilitates the cooling of the pitch which is spread on the belt. The belt is supported on the pulley members 6 and 7. The pulley 7 75 is driven by the motor 8, thru a suitable transmission 9. The pulley 6 is rotatably mounted on a suitable shaft supported by the framework 10, which is adapted to slide upon the bases 11. The frame-work is connected to the counter-weight 12 by the cable 13 which works over the pulley 14. By proper weighting of the counterweight the proper tension 80 is always maintained upon the belt. Expansion and contraction of the metal belt are 85 compensated for by movement of the framework 10 upon the bases 11.

The lower portion of the belt is supported by idlers 15 mounted in suitable journal boxes 90 in the supports 16.

The upper portion of the belt is maintained level by the idlers 17 suitably mounted in bearings 18 which may, for example, be supported outside of the trough 19 as shown 95 in Fig. 3.

With the trough are sprays 20 supplied with water from the line 21 and directed against the under-side of the upper portion of the belt. Instead of water any other suitable cooling or refrigerating medium may be employed. The trough serves to confine, and also to collect, the spray, that portion which is not volatilized being collected in the bottom of the trough and drained off thru the pipes 22.

The pitch is run on to the belt from the pitch trough 23. The trough may be provided with a jacket 23' as shown in Fig. 3, which serves to insulate the trough, or means may be provided for circulating a hot gas 100 thru the jacket where this is necessary to insure that the pitch is brought to the belt in a thinly fluid condition. The flow of pitch and the speed of travel of the belt are advantageously adjusted so that the pitch 105 spreads upon the belt in a relatively thin layer. The rate at which the pitch is fed to the belt and the rate at which the belt travels and the length of the belt and the cooling action are so controlled that the pitch is chilled and brought into such a brittle condition before leaving the belt that it is easily fractured. The drawing shows a hopper 24 for collecting the pitch as it is discharged from the belt as the belt passes around the pulley 7. 110

The pitch may be collected from the belt as the belt passes over the pulley 7 or side discharge means may be provided for removing the pitch from the belt before it reaches the pulley 7. Such means may comprise a 115

scraper positioned at an angle of 45° to the direction of travel of the belt. As the pitch comes in contact with such a scraper it will be discharged from the side of the belt.

5 In order to prevent water used for cooling the belt from collecting in the hopper together with the pitch, wipers 26 are advantageously provided to remove adhering particles of water from the under-side of the belt before it reaches the pulley 7. These 10 wipers may comprise rubber strips 26 held in a slot in the pipe 27. The water which is removed from the belt by these wipers is collected in the trough 19 and drains thru the 15 outlets 22 with other excess water from the sprays.

In a typical case pitch from coke oven tar having a melting point of about 400° F. was delivered to the belt at a temperature of about 20 350° C. and was allowed to spread freely thereon. The width of the belt was about 18" and the distance from the point at which the pitch came onto the belt and the point at which it was discharged from the belt was 25 about 57 feet. The driving mechanism was regulated so that the speed of travel of the belt was about fifty feet per minute. This gave a cooling period of about sixty-eight seconds and under these conditions the pitch 30 which, when cooled, gave a flake about one-tenth of an inch thick, was chilled and cracked to some extent on the belt and was broken into small flakes as it fell from the conveyor and was collected in the hopper. 35 Thin, small, brittle flakes of pitch were obtained. The belt handled in the neighborhood of 160 gallons of pitch per hour.

The length of the belt may be varied to provide more or less cooling of the pitch and the 40 rate at which the belt travels may also be controlled to regulate the length of time during which the pitch is held on the belt. Various means for cooling the belt with air coolers and other cooling devices may be employed 45 but spraying the underside of the belt with water will be sufficient to provide the cooling required to solidify hard pitches. The temperature to which the pitch must be cooled before being discharged from the belt depends upon the melting point of the pitch; 50 higher melting point pitches become solid at higher temperatures, and lower melting point pitches require cooling to lower temperatures in order to effect solidification.

55 The pitch is ordinarily fed on to the conveyor in such a way as to form a thin layer of the pitch. Ordinarily a relatively narrow ribbon of the pitch is formed in order that the pitch on solidifying will readily break into 60 small chips or flakes. A wider ribbon or sheet of pitch may be formed by allowing pitch to flow on to the same belt from several adjacent sources. Various means of forming such a wider sheet of the pitch may be devised. 65 Several narrower ribbons of pitch may gen-

erally be preferred to one broader sheet of the pitch in order to facilitate breaking the pitch into bits. A wider belt may be employed and several separate streams of pitch may be run on to the belt in such a way as to form 70 several separate parallel ribbons of pitch on the single belt.

The apparatus herein described is simple and the operation is also simple. There are no complicated units and the method of operation is free from involved steps. The cost of installing such a pitch-flaking apparatus is small and the cost of operating it is not large. The invention provides a method of 75 producing small particles of hardened pitch without the necessity of grinding or otherwise comminuting large lumps or chunks, and is desirable for this and other reasons.

This application is in part a continuation of my co-pending application Serial No. 227,927, 80 filed October 22, 1927.

I claim:

The method of flaking pitch which comprises discharging the pitch in the form of a hot molten stream, forming the said stream 90 into a ribbon-like thin layer, subjecting one side of the layer to a cooling medium until it is sufficiently brittle to be readily broken and then breaking said ribbon-like layer of pitch and causing said resulting fragments to drop 95 whereby they will be broken into flakes as they fall onto the receiving means.

In testimony whereof I affix my signature.

STUART PARMELEE MILLER.

100

105

110

115

120

125

130